

July 22, 1969

J. I. JOHANSSON

3,456,831

## AUSTENITIC STAINLESS STEEL PRESSURE VESSELS

Original Filed Sept. 20, 1963

6 Sheets-Sheet 1



INVENTOR.  
JOHAN INGVAR JOHANSSON

BY

Brumbaugh, Free, Graves & Donohue  
his ATTORNEYS

July 22, 1969

J. I. JOHANSSON

3,456,831

AUSTENITIC STAINLESS STEEL PRESSURE VESSELS

Original Filed Sept. 20, 1963

6 Sheets-Sheet 2



FIG. 4A



FIG. 4B

INVENTOR  
JOHAN INGVAR JOHANSSON

BY

Brumbaugh, Free, Graves & Donohue  
his ATTORNEYS

July 22, 1969

J. I. JOHANSSON

3,456,831

AUSTENITIC STAINLESS STEEL PRESSURE VESSELS

Original Filed Sept. 20, 1963

6 Sheets-Sheet 3



FIG. 5A



FIG. 5B

INVENTOR  
JOHAN INGVAR JOHANSSON

BY

Brumbaugh, Free, Graves + Donohue

his ATTORNEYS

July 22, 1969

J. I. JOHANSSON

3,456,831

AUSTENITIC STAINLESS STEEL PRESSURE VESSELS

Original Filed Sept. 20, 1963

6 Sheets-Sheet 4

AVERAGE TIME TO STRESS CORROSION FAILURE IN 40 %  $\text{CaCl}_2$ ,  
pH 6, 100°C AFTER DIFFERENT DEGREE OF COLD STRETCHING.  
UNIAXIAL TENSION, APPLIED STRESS =  $2/3 \sigma_{0.2}$  AT 100°C.  
TEST STEEL - AVESTA 832 SK.



FIG. 7



FIG. 6

INVENTOR  
JOHAN INGVAR JOHANSSON

BY

Brumbaugh, Free, Grace & Donohue  
his ATTORNEYS

July 22, 1969

J. I. JOHANSSON

3,456,831

AUSTENITIC STAINLESS STEEL PRESSURE VESSELS

Original Filed Sept. 20, 1963

6 Sheets-Sheet 5

ACCELERATED STRESS CORROSION TESTS IN 40 %  $\text{CaCl}_2$ ,  
100°C USING UNIAXIAL CONSTANT TENSION OF 15  $\text{kg/mm}^2$ .  
TEST STEEL-COLD STRETCHED AVESTA 832 MV.



FIG. 8

ACCELERATED STRESS CORROSION TESTS IN 40 %  $\text{CaCl}_2$ ,  
100°C USING UNIAXIAL TENSION =  $2/3 \sigma_{0.2}$ .  
TEST STEEL-AVESTA 832 MV.



FIG. 9

INVENTOR,  
JOHAN INGVAR JOHANSSON

BY

*Brumbaugh, Frey, Graves & Donohue*  
his ATTORNEYS

July 22, 1969

J. I. JOHANSSON

3,456,831

AUSTENITIC STAINLESS STEEL PRESSURE VESSELS

Original Filed Sept. 20, 1963

6 Sheets-Sheet 6

FIG. 10

MECHANICAL PROPERTIES BETWEEN +20 AND 400°C  
OF AVESTA 832 SK STAINLESS STEEL-COLD STRETCHED



INVENTOR  
JOHAN INGVAR JOHANSSON

BY

*Brumbaugh, Free, Graves + Donohue*

his ATTORNEYS

1

3,456,831  
**AUSTENITIC STAINLESS STEEL  
PRESSURE VESSELS**

Johan Ingvar Johansson, Avesta, Sweden, assignor to  
Avesta Jernverks Aktiebolag, Avesta, Sweden, a corporation of Sweden

Continuation of application Ser. No. 310,383, Sept. 20, 1963, which is a continuation-in-part of application Ser. No. 754,598, Aug. 12, 1958. This application Jan. 20, 1967, Ser. No. 610,713

Claims priority, application Sweden, Aug. 16, 1957,

7,520/57

Int. Cl. B65d 1/00, 7/42

U.S. Cl. 220—3

8 Claims

## ABSTRACT OF THE DISCLOSURE

Austenitic stainless steel pressure vessels are made by welding together a plurality of plates of austenitic stainless steel having a normal yield strength with weldments of austenitic stainless steel to form a pressure vessel, selecting a higher than normal value of yield strength within a range of values provided by cold stretching the steel an amount sufficient to elongate it permanently essentially in excess of 0.2% and at most about 10%, and subjecting the vessel internally to a fluid pressure sufficient to stress the weakest portions of the vessel walls to the selected yield strength and thereby increase the yield strength of the said weakest portions to the selected value by permanently elongating the said weakest portions of the walls essentially in excess of 0.2% and at most about 10%, the vessel being subjected to the fluid pressure at a temperature below the recrystallization temperature of the steel and under conditions permitting the vessel walls to expand freely.

This is a continuation of Ser. No. 310,383 filed Sept. 20, 1963 and now abandoned, which in turn is a continuation-in-part of Ser. No. 754,598, filed Aug. 12, 1958, and now abandoned.

This invention relates to welded pressure vessels formed of austenitic stainless steels.

Pressure vessels, including sealed vessels such as autoclaves and gas containers, and also long open vessels which are subjected to high static pressures from liquid columns, preferably are formed of materials that are highly stress and corrosion resistant. Those characteristics are possessed by austenitic stainless steels which are, therefore, ideally suited to high pressure vessels.

Due to the high relative cost of austenitic stainless steels, when the nature of corrosive material to be held in a container required their use, it was more economical, prior to the invention, to use stainless clad ferritic steel plates than to use solid stainless steel plates. Various problems associated with the construction and use of vessels formed of clad steel plates made it desirable to use solid stainless steel, if possible. Only the high cost of those steels has prevented their use in many pressure vessels.

One disadvantage of stainless steels, and particularly those stainless steels having a composition including approximately 18% chromium and about 8 to 12% nickel which have austenite as an essential structural constituent, is their lack of a marked yield point and the low value of the yield strength arbitrarily selected relative to the ultimate tensile strength. Various governmental and other safety codes ordinarily have provisions governing

2

wall thickness of pressure vessels dependent on the yield strength of stainless steels, as well as their other properties, and the relatively low yield strength selected makes necessary thick vessel walls of expensive stainless steel.

In contrast, ferritic type low alloy steels often used in pressure vessels have a marked yield point which enables the yield strength used to calculate wall thickness to be set almost precisely at the yield point. This value can be defined as the stress which in a tensile test gives a certain elongation without any further increase in stress. However, for materials such as austenitic stainless steels having no marked yield point, a relatively low value for the yield strength has been used in safety codes to calculate wall thickness of pressure vessels.

15 The present invention overcomes the disadvantages formerly associated with the use of austenitic stainless steels in pressure vessels by providing thinner wall stainless steel vessels with great savings, for example, up to and even greater than one-half of the amount of stainless steel formerly required for the vessels.

20 In one embodiment of the invention, sections of stainless steel having austenite as an essential structural constituent, hereinafter referred to as austenitic stainless steel, are welded to form a pressure vessel of the desired shape. The vessel is then subjected internally to fluid pressure, under conditions permitting the vessel walls to expand freely, sufficient to provide a desired yield strength higher than the normal yield strength by cold stretching the vessel walls to cause a permanent elongation in excess of 0.2% and at most 10% in the weakest regions of the walls at a temperature below the recrystallization point of the steel. The cold stretching of the austenitic stainless steel preferably is sufficient to increase its yield strength at room temperature from 15 to 100%, the final 35 yield strength being high enough to withstand established working pressures with a prescribed margin of safety. Free expansion of the vessel walls is necessary to effect permanent elongation in all required parts of the vessel.

30 The resulting inventive pressure vessel, which is formed of a plurality of cold stretched sections welded together, has a markedly higher yield strength for the amount of stainless steel used in its walls. Moreover, stresses at welds between the vessel sections are relieved by the cold stretching, thereby reducing the danger of weld fracture. It has also been found that, contrary to the general opinion of those in the pressure vessel field, stress corrosion resistance of the vessel is not significantly impaired by cold stretching within the limits of the invention and, in some instances, vessels have shown, after being permanently elongated essentially in excess of 0.2% and at most 10%, improved stress corrosion resistance.

35 When it is necessary to reduce the amount of distortion of the pressure vessel due to cold stretching, pursuant to another embodiment of the invention, the austenitic stainless steel sections are cold stretched, cold rolled or otherwise cold worked, at a temperature below the recrystallization point of the steel, to raise their yield strength to a selected value prior to being welded together to form the pressure vessel. Subsequently, pressure is applied to the vessel internally to cold stretch the weld joints and adjacent annealed areas essentially in excess of 0.2% and at most 10%, thereby raising the yield strength of the weakest regions of the vessel to the desired value while reducing to a negligible value distortion 50 of the vessel.

40 If it is necessary to weld pipe sockets, manhole fittings and similar connections to the vessel after the cold

stretching, annealing effects at the weldments and adjacent areas can be compensated by suitably reinforcing such connections. Alternatively, those regions where fittings are to be positioned can initially be designed with larger dimensions than the surrounding portions to provide sufficient strength so that no elongation therein is

of standard stainless steels having austenite as an essential structural constituent produced by Avesta Jernverks Aktiebolag of Sweden and their equivalent steels designated by other Swedish, American, British and German code numbers. The table also shows the statistical yield strength ( $\sigma_{0.2}$ ) of the steels at room temperature (20° C.).

TABLE 1

| Avesta Grade | Swedish SIS | American AISI | British En | German Wst. Nr. | Statistical yield strength ( $\sigma_{0.2}$ ) at 20° C. |
|--------------|-------------|---------------|------------|-----------------|---------------------------------------------------------|
| 832 M        | 2,832       | 302           | 58E        | 4,300           | 24 kg./mm. <sup>2</sup>                                 |
| 832 MV       | 2,833       | 304           | (58E)      | 4,301           | 24 kg./mm. <sup>2</sup>                                 |
| 832 MVR      |             | 304L          |            | 4,306           | 23 kg./mm. <sup>2</sup>                                 |
| 832 MVT      | 2,837       | 321           | 58B/58C    | 4,541           | 25 kg./mm. <sup>2</sup>                                 |
| 832 SK       | 2,843       | 316           | 58J        |                 | 27 kg./mm. <sup>2</sup>                                 |
| 832 SKR      |             | 316L          |            | 4,435           | 25 kg./mm. <sup>2</sup>                                 |
| 832 SKT      | 2,844       |               | 58J        | 4,573           | 27 kg./mm. <sup>2</sup>                                 |
| 832 SN       |             |               | 317        |                 | 28 kg./mm. <sup>2</sup>                                 |

necessary and none will result during the stretching treatment.

These and further advantages of the invention will be more readily understood when the following description is read in conjunction with the accompanying drawings, in which:

FIGURE 1 is a sectional view of a welded cylindrical pressure vessel formed of austenitic stainless steel prior to permanent elongation;

FIGURE 2 illustrates the pressure vessel of FIGURE 1 after it has been cold stretched and fittings added;

FIGURE 3 shows another pressure vessel constructed in accordance with the present invention;

FIGURES 4A and 4B illustrate stress-strain curves for an austenitic stainless steel and ferritic steels;

FIGURES 5A and 5B show stress-strain curves for the austenitic stainless steel of FIGURES 4A and 4B after cold stretching;

FIGURE 6 illustrates curves comparing the ultimate tensile strength and yield strength of an austenitic stainless steel as it is cold stretched;

FIGURES 7, 8 and 9 illustrate the stress corrosion characteristics of austenitic stainless steels that have been cold stretched in varying amounts; and

FIGURE 10 shows graphically the mechanical properties of an austenitic stainless steel between 20° C. and 400° C. after cold stretching varying amounts.

Referring to a typical pressure vessel constructed in accordance with the present invention with reference to FIGURES 1 and 2, a pair of domed end walls 10 and 11 are welded to the ends of a cylindrical shell 12 at circumferential weldments 13 and 14. The shell 12 may be formed of two sections welded together at a weldment 15. One or more longitudinal weldments (not shown) in the shell facilitate construction of the pressure vessel.

Circular apertures in the center of each of the end walls 10 and 11 receive cylindrical pipe sockets 16 and 17, respectively, and two cylindrical pipe sockets 18 and 19 are also welded into circular apertures provided on opposite sides of the shell 12. The pipe sockets 16, 17, 18 and 19 are temporarily sealed by welding domed covers 20, 21, 22 and 23, respectively, over their open ends. Centrally of one of the covers, shown as the cover 20, a smaller connecting pipe 24 is welded to receive a suitable connection from a source of fluid under pressure such as a high pressure water pump (not shown).

The end walls 10 and 11, and the shell 12, are formed of an austenitic stainless steel including about 18% chromium and 10% nickel. Eight to fourteen percent nickel has also been used and the particular proportions depend on the exact end use of the vessel. Such steels are normally referred to as 18-8 stainless steels. The highly acid resistant steels also contain from 1.5 to 4.5% molybdenum. The following Table 1 sets forth a number

In addition to possessing the characteristics of high resistance to corrosion, the steels listed in Table 1 possess excellent properties from a constructional point of view. Their tensile strength is good, elongation extraordinarily good and impact strength excellent. Their relatively low yield strength in the as-delivered condition is, however, disadvantageous. Thus, when calculating the thickness of walls necessary for a pressure vessel, the calculations must be based on a standardized yield strength value prescribed for the grade steel that is to be used in the pressure vessels. The low yield strengths designated for these stainless steels has made necessary the use of walls uneconomically thick.

Using steels of the ferritic type; i.e., ordinary low alloy pressure vessel steels which have a more or less marked yield point, the yield stress in accordance with the generally adopted code definitions is set equal to the lower yield point. This value can be defined as the stress in which a tensile test gives a certain elongation without any increase in stress.

Since the austenitic stainless steels have no marked yield point, the so-called  $\sigma_{0.2}$  value, the stress that gives 0.2% permanent elongation of the material, is used as the basis for calculating a code yield strength.

The foregoing is made evident by considering FIGURES 4A and 4B which illustrate stress-strain curves of two typical pressure vessel ferritic steels SIS 1330 and SIS 2101 and an austenitic stainless steel grade Avesta 832 SK. Since the scale of FIGURE 4A is so small that the differences in the initial portions of the curves cannot be observed, the strain scale has been greatly enlarged in FIGURE 4B to show in detail the yield point of the ferritic steels and the absence of any marked yield point for the austenitic stainless steel. Thus, the SIS 1330 and SIS 2101 steels show marked yield points at 26 and 34 kg./mm.<sup>2</sup>, respectively, while the curve for the Avesta 832 SK steel shows no marked yield point. Note that the  $\sigma_{0.2}$  value for the specimen plotted is approximately 28 kg./mm.<sup>2</sup>.

Beyond the yield points of the low alloy ferritic steels in FIGURE 4B, the stress-strain curves for the ferritic and austenitic steels differ greatly in shape. The low alloy ferritic steels first undergo a significant elongation without increase in stress (dashed portions of curves) and then their curves turn sharply up, leveling out soon thereafter. The highest stress calculated from the original cross-section which these steels can withstand; i.e., their ultimate tensile strength, is reached after only about 20% strain. Following this maximum point, a local contraction occurs and the specimens fracture.

Examining the curve of the austenitic steel, the material shows a marked strain hardening rate from the very beginning and the maximum stress; i.e., the ultimate tensile strength, is reached at a strain of about 50%. Note that

the ultimate tensile strength of this steel is substantially higher than that of the low alloy ferritic steels.

The curve of FIGURE 4B also shows that austenitic stainless steel tends to harden very rapidly when deformed at room temperature; i.e., at a temperature below its recrystallization point. Thus, permanent elongation of only about 5% results in a yield strength increase of about 15 kg./mm.<sup>2</sup>. This increase does not appreciably reduce the elongation characteristics or the impact strength value of the steel. Referring to FIGURES 5A and 5B, which show on two scales stress-strain curves for the Avesta 832 SK steel after having been cold stretched 5%, note that the  $\sigma_{0.2}$  value is approximately 17 kg./mm.<sup>2</sup> higher than for the unstretched material shown in FIGURES 4A and 4B.

Prior to the present invention, the wall thickness of the pressure vessel shown in FIGURE 1 had been determined by using a calculating value for the yield strength ( $\sigma_{ber}$ ) found in the Swedish Pressure Vessel Code. The following table lists the calculating values for pressure vessels formed of various steels, including a low alloy ferritic steel 1430 when the wall thickness is 30 mm. or less, and four austenitic stainless steels designated both by the Avesta grade and the Swedish SIS number.

TABLE 2.—CALCULATING VALUES FOR THE YIELD STRENGTH ( $\sigma_{ber}$ ) ACCORDING TO THE SWEDISH PRESSURE VESSEL CODE

| Temp.,<br>°C. | Steel Grade             |                |                 |                |                 |
|---------------|-------------------------|----------------|-----------------|----------------|-----------------|
|               | 1430<br>S $\leq$ 30 mm. | 832 MV<br>2333 | 832 MVT<br>2333 | 832 SK<br>2343 | 832 SKT<br>2343 |
| 20            | 23.0                    | 20.0           | 20.0            | 21.0           | 22.0            |
| 50            | 23.0                    | 18.0           | 18.5            | 18.9           | 20.8            |
| 75            | 23.0                    | 16.8           | 17.6            | 17.6           | 20.0            |
| 100           | 23.0                    | 15.5           | 16.7            | 16.2           | 19.1            |
| 125           | 23.0                    | 14.8           | 16.1            | 15.4           | 18.5            |
| 150           | 23.0                    | 14.0           | 15.6            | 14.6           | 17.8            |
| 175           | 22.5                    | 13.5           | 15.3            | 14.0           | 17.4            |
| 200           | 22.0                    | 12.9           | 14.7            | 13.5           | 17.0            |
| 225           | 21.0                    | 12.5           | 14.3            | 13.1           | 16.7            |
| 250           | 19.5                    | 12.1           | 14.0            | 12.7           | 16.4            |
| 275           | 18.0                    | 11.8           | 13.7            | 12.8           | 16.2            |
| 300           | 16.5                    | 11.4           | 13.4            | 12.0           | 16.0            |
| 325           | 14.0                    | 11.2           | 13.2            | 11.8           | 15.8            |
| 350           | 10.9                    | 13.0           | 11.5            | 15.6           |                 |
| 375           | 10.7                    | 12.8           | 11.3            | 15.4           |                 |
| 400           | 10.5                    | 12.6           | 11.0            | 15.2           |                 |

The calculating value  $\sigma_{ber}$  for each grade of steel is lower than the statistical value for the yield strength  $\sigma_{0.2}$  to insure that it encompasses all melts of the particular steels. For example, while the yield strength of the Avesta 832 SK specimen shown in FIGURES 4A and 4B is representative of the statistical normal yield strength  $\sigma_{0.2}$  of this grade, other specimens may have yield strengths as low as 20 or 21 kg./mm.<sup>2</sup>. Safety codes must allow for such variances when concerned with high pressure vessels even though the low calculating values  $\sigma_{ber}$  make necessary the use of excessive amounts, in certain instances, of expensive 18-8 stainless steel.

According to the invention, the wall thickness of the pressure vessel shown in FIGURE 1 is calculated using a selected higher yield strength  $\sigma_k$ , for example 30 kg./mm.<sup>2</sup>, which is substantially higher than the calculating value for yield strength ( $\sigma_{ber}$ ) specified by the Pressure Vessel Code, and which is also higher than the statistical normal yield strength ( $\sigma_{0.2}$ ) of the steel. This results in a calculated requirement of substantially thinner walls in the vessel with a resultant significant saving of expensive stainless steel. The pressure necessary to cold stretch the vessel walls to obtain the selected yield strength is then calculated and the vessel subsequently stretched. A typical calculation to satisfy the Swedish Pressure Vessel Code for a vessel formed of Avesta 832 MV (equivalent to American AISI 304) is set forth in the following example.

### Example I

Assuming the requirement of a pressure vessel in the category of a thin-walled vessel with an inner diameter of 2000 mm. that is to be subjected to a 12 atmospheres overpressure at a temperature of 20° C., and formed of Avesta 832 MV austenitic stainless steel, according to the Code formula

$$s_{min.} = \frac{D_i \times p}{200 \times \sigma_{ber} \times S_F \times z}$$

where

- 15  $s_{min.}$ =minimum wall thickness of the vessel shell in mm.  
 $D_i$ =inner diameter of the vessel in mm.  
 $p$ =working pressure in atmospheres overpressure  
 $\sigma_{ber}$ =calculating value for the yield strength of the material at its use temperature in kg./mm.<sup>2</sup> (see Table 2)  
20  $S_F$ =safety factor=1.5  
 $z$ =joint efficiency=0.9 for X-ray controlled joints  
According to the Code,  $\sigma_{ber}=20$  kg. per mm.<sup>2</sup> (from Table 2; note that the yield strength  $\sigma_{0.2}=24$  kg./mm.<sup>2</sup> from Table 1). Therefore

25

$$s_{min.} = \frac{2000 \times 12 \times 1.5}{200 \times 20.0 \times 0.9}$$

$$s_{min.} = 10.0 \text{ mm.}$$

These calculations show that a conventional pressure vessel formed of Avesta 832 MV steel must have a minimum wall thickness of 10 mm. to satisfy the requirements of the Swedish Code.

A higher yield strength value  $\sigma_k$  is then selected, in this instance 30 kg./mm.<sup>2</sup>, to permit the calculating value  $\sigma_{ber}$  to be increased to 30 kg./mm.<sup>2</sup>. Again computing wall thickness with  $\sigma_{ber}=30$

40

$$s_{min.} = \frac{2000 \times 12 \times 1.5}{200 \times 30 \times 0.9}$$

$$s_{min.} = 6.7$$

45 And rounding off

$$s_{min.} = 7 \text{ mm.}$$

Constructing the pressure vessel with a wall thickness of 7 mm. uses 30% less steel than would be required for a vessel constructed with a wall thickness of 10 mm.

50 Next the pressure  $P_k$  necessary to cold stretch the sealed pressure vessel to increase its yield strength to 30 kg./mm.<sup>2</sup> is calculated. The formula for calculating  $P_k$ , which provides wall stresses in the vessel equal to the desired yield strength, is in principle the same as for calculating wall thickness. However, the safety factor and joint efficiency may be disregarded and 1 substituted therefor. Therefore, the basic formula for thin-walled vessels is

55

$$(2) \quad P_k = \frac{s \times \sigma_k \times 200}{D_i}$$

where

- 65  $s$ =actual wall thickness of the vessel shell in mm.  
 $\sigma_k$ =the desired yield strength of the steel in kg./mm.<sup>2</sup>  
 $D_i$ =the inside diameter of the shell

70 Therefore

$$P_k = \frac{7 \times 30 \times 200}{2000}$$

$$P_k = 21 \text{ kg./cm.}^2$$

75

According 21 kg./cm.<sup>2</sup> is the fluid pressure required to cold stretch the vessel sufficiently, about 2% in the weakest regions of the vessel in this instance, to provide a yield strength  $\sigma_k$  of 30 kg./mm.<sup>2</sup>. Of course, thicker portions of the vessel will be less affected, and in some instances unaffected, by the cold stretching. However, because the vessel is permitted to expand freely, the weakest regions will be stretched the greatest amount and will, therefore, increase more in yield strength than other portions of the vessel.

Applying these calculations to the vessel of FIGURE 1, after it has been welded together with relatively thin walls, a high pressure water source is connected to the pipe 24 and the pressure in the vessel is increased in stages to the pressure of 21 kg./cm.<sup>2</sup> to cold stretch the walls of the vessel sufficiently to obtain a minimum yield strength of 30 kg./mm.<sup>2</sup>. Even though the vessel expands freely, its walls will be shaped substantially the same as the original unstretched vessel. Thus, the yield strength of the austenitic stainless steel in its stretched area increases rapidly and the initially weakest regions first subjected to stretching increase in yield strength to such an extent that comparatively quickly the stretching spreads to other portions of the vessel.

Control measurements may also be carried out as the pressure is increased on the change of circumference of the vessel. Note that the end portions of the shell 12 will be stretched slightly less than other regions since they are lent support by the domed walls 10 and 11. Also reinforced and overdimensioned portions and those portions which because of their location in the vessel will not be subjected to sufficiently high stresses, will be stretched little or not at all. The same also holds true for those portions which already have the necessary yield strength. Therefore the circumference will not change precisely the same percentage as the weakest regions of the vessel.

When the cold stretching is completed, the temporarily welded covers 20, 21, 22 and 23 are cut off and, in the example shown in FIGURE 2, ribbed pipes 25 and 26 are welded to the pipe sockets 16 and 17, a straight pipe 27 is welded to the socket 18, and a flanged elbow pipe 28 is welded to the socket 19.

Since the sockets 16 and 18 are formed of relatively thin material, the adjacent vessel walls are reinforced by extra welded sheet metal plates 16a and 18a. On the other hand, the pipe sockets 17 and 19 are sufficiently strong to stiffen the adjacent portions of the vessel walls and compensate for weakening due to the socket apertures.

When it is desirable to weld a pipe socket to a pressure vessel subsequent to cold stretching, a reinforcement with sufficient thickness to compensate for the heating and annealing effects during the subsequent welding may form a portion of the vessel. Thus, the shell 12 of FIGURES 1 and 2 includes a plate 29 that is considerably thicker than the remaining plates. Subsequent to cold stretching of the vessel, an opening is cut in the plate 29 and a manhole fitting 30 welded into the opening, as shown in FIGURE 2. The manhole fitting is dimensioned to compensate for weakening due to the aperture, and the thickness of the plate 29 is chosen to compensate for the decrease in yield strength caused by the welding operation. A manhole cover 31 is held in place by a crossbar 32 joined to the cover by a nut and bolt 33.

## EXAMPLE II

Considering another exemplary pressure vessel constructed in accordance with the invention, assuming a thin-walled shell having an inner diameter of 6000 mm. to be subjected to 4 atmospheres overpressure at a temperature of 100° C., and formed of Avesta 832 SK steel (equivalent to American AISI 316), according to the

Swedish Pressure Vessel Code,  $\sigma_{ber}=16.2$  (from Table 2). Substituting in Formula 1

$$s_{min.} = \frac{6000 \times 4 \times 1.5}{200 \times 16.2 \times 0.9}$$

$$s_{min.} = 12.3 \text{ mm.}$$

Thus a conventional pressure vessel formed of Avesta 832 SK steel requires walls 12.3 mm. thick.

A higher yield strength value  $\sigma_k$  of 35 kg./mm.<sup>2</sup> is then selected. However, since the vessel will be cold stretched at 20° C., this yield strength value must be converted to a value that may be used in Formula 1. Table 2 shows that at 20° C. the calculating value  $\sigma_{ber}$  is 21 kg./mm.<sup>2</sup> and at 100° C. the value is 16.2 kg./mm.<sup>2</sup>. Referring to FIGURE 10, which shows the mechanical properties of Avesta 832 SK steel at temperatures ranging from 20° C. to 400° C. after cold stretching varying amounts, it is apparent that a direct ratio cannot be made to obtain the higher yield strength necessary at 20° C. to provide the selected yield strength at 100° C. Because the curves for 0%, 2.5%, etc. have generally the same contours, the value can be obtained by calculating the difference between the selected yield strength at 100° C. and the code yield strength at 100° C., which is 35 minus 21=14 kg./mm.<sup>2</sup>, and adding this amount to the code yield strength at 100° C.; thus 16.2 plus 14=30.2 kg./mm.<sup>2</sup>. Substituting a calculating value of 30.2 kg./mm.<sup>2</sup> in Formula 1

$$s_{min.} = \frac{6000 \times 4 \times 1.5}{200 \times 30.2 \times 0.9}$$

$$s_{min.} = 6.6 \text{ mm.}$$

And rounding off

$$s_{min.} = 7 \text{ mm.}$$

Constructing the vessel with a wall thickness of 7 mm. results in a saving of about 43% of the steel used in a conventional vessel having a wall thickness of 12.3 mm.

Next the pressure  $P_k$  necessary to cold stretch the sealed pressure vessel to increase its yield strength to 35 kg./mm.<sup>2</sup> at 100° C. (30.2 kg./mm.<sup>2</sup> at 20° C.) is calculated by substituting in Formula 2

$$P_k = \frac{7 \times 30.2 \times 200}{6000}$$

$$P_k = 7 \text{ kg./cm.}^2$$

Therefore 7 kg./cm.<sup>2</sup> is the fluid pressure required to cold stretch the vessel sufficiently, about 2%, in the weakest regions of the vessel, to provide a yield strength ( $\sigma_{0.2}$ ) at 100° C. of 35 kg./mm.<sup>2</sup>.

It is apparent from Example II and FIGURE 10 that austenitic stainless steels provide, when cold stretched, higher yield strengths at elevated temperatures as well as at room temperature. Tests show that prolonged heating does not impair the higher yield strengths obtained at elevated temperature. Note also that the real yield strength increase remains practically unchanged at different temperatures and, therefore, the relative yield strength increase is higher at elevated temperatures. This enables great savings in the amount of stainless steel used as is illustrated by Example II.

Examples I and II demonstrate in detail how the principles of the present invention are applied to the construction of austenitic stainless steel pressure vessels under the applicable Swedish Code. The following Examples III, IV and V compare the manner of calculating the wall thickness of the inventive pressure vessels pursuant to the Swedish Pressure Vessel Code, 1959, Berechnung von Druckbehältern, AD-Merkblatt B1, August 1959 (West Germany) and ASME Boiler and Pressure Vessel Code, Section VIII, 1962. The following Table 3 shows the designations used in the different Codes as well as some basic formulas of calculation.

TABLE 3

| Definition                                       | Designations and formulas                                                  |                                               |                                            |
|--------------------------------------------------|----------------------------------------------------------------------------|-----------------------------------------------|--------------------------------------------|
|                                                  | Swedish Pressure Vessel Code                                               | German AD-Merkblatt B1                        | ASME                                       |
| Minimum thickness of shell                       | $s_{min.}$ , mm.                                                           | S, mm.                                        | t, inches.                                 |
| Design pressure                                  | $p$ , kg./cm. <sup>2</sup>                                                 | $p$ , kg./cm. <sup>2</sup>                    | $P$ , p.s.i.                               |
| Radius of the shell:                             |                                                                            |                                               |                                            |
| Inside                                           | $D/2$ , mm.                                                                | $D/2$ , mm.                                   | R, inches.                                 |
| Outside                                          |                                                                            | $D/2$ , mm.                                   |                                            |
| Safety factor                                    | $SF = 1.5$                                                                 | $s = 1.5$                                     | Included in the allowable stress.          |
| Maximum allowable stress                         | $\sigma_{ber}/SF$ , kg./mm. <sup>2</sup>                                   | K/s, kg./mm. <sup>2</sup>                     | S, p.s.i.                                  |
| Joint efficiency                                 | $z$                                                                        | v                                             | E.                                         |
| At temp. < 120° C.                               |                                                                            |                                               |                                            |
| Basic formula for thin-walled cylindrical shells | $s_{min.} = \frac{D \times p}{200 \times \sigma_{ber} \times z \times SF}$ | $S = \frac{D \times p}{200 K/s \times v}$     | $t = \frac{P \times R}{S \times E + 0.6P}$ |
| At temp. > 120° C.                               |                                                                            |                                               |                                            |
|                                                  |                                                                            | $S = \frac{D \times p}{200 K/s \times v + p}$ |                                            |

The three basic formulas of calculation in Table 3 are identical in principle, although there are some different factors. In Sweden the maximum joint efficiency is 0.9 but in West Germany and the United States a joint efficiency of 1 may be used. Since the material costs of stainless steel vessels are comparatively high, all calculations have been made with maximum joint efficiencies.

In Sweden and Germany the pressure vessel dimensions are based on the yield strength of the material. By using a safety factor which in both cases is 1.5, the allowable stress is limited to  $\frac{2}{3}$  of the stated calculating value for the yield strength. However, the ASME code indicates directly the allowable stress which has been based on the ultimate tensile strength of the material in such a way that the allowable stress is 25% of the ultimate tensile strength.

When calculations are based on the yield strength, the increased yield strength value provided by using the inventive cold stretching method is used in the formula. The cold stretching pressure ( $P_k$ ) required to provide the higher yield strength is so chosen that the resulting wall stress in the vessel is equal to such yield strength. The formula for calculating  $P_k$  has been given as Formula 2 in Example I for thin-walled vessels in Sweden.

In a thick-walled vessel the stress distribution is somewhat more complicated; for that reason special formulas are used for calculation of the shell thickness. The calculation of  $P_k$  is also based on those special formulas in a similar way as shown above in Example I.

Different codes designate various allowable stresses for austenitic stainless steel. Table 2 shows in detail the Swedish Code calculating values and the following Table 4 compares, for Avesta 832 MV and 832 SK steels, the Swedish, German and interpolated ASME Code values. Specifically, the Swedish and German values below correspond to the calculating values in the Swedish Pressure Vessel Code and AD-Merkblatt W2 1956, respectively. However, the code values have been reduced to  $\frac{2}{3}$  (safety factor) in order to correspond to the allowable stress and thus be comparable with the ASME values.

20

TABLE 4

| Steel Type | Avesta 832 MV,<br>SIS 2333 | Werkstoff 4301                                           |                                                                          | AISI 304                        |                      |
|------------|----------------------------|----------------------------------------------------------|--------------------------------------------------------------------------|---------------------------------|----------------------|
|            |                            | Swedish Pressure Vessel Code                             | AD-Merkblatt W2 Streckgrenze $\times \frac{2}{3}$ , kg./mm. <sup>2</sup> | ASME Code (Interpolated values) | Kg./mm. <sup>2</sup> |
| 25         | Temperatures               | $\sigma_{ber} \times \frac{2}{3}$ , kg./mm. <sup>2</sup> | $\times \frac{2}{3}$ , kg./mm. <sup>2</sup>                              |                                 |                      |
|            | °C. °F.                    |                                                          |                                                                          |                                 |                      |
|            | 20 68                      | 13.3                                                     | 14.7                                                                     | 13.2                            | 18,750               |
|            | 50 122                     | 12.0                                                     | 13.0                                                                     | 12.8                            | 18,270               |
|            | 100 212                    | 10.3                                                     | 11.3                                                                     | 11.8                            | 17,850               |
|            | 150 302                    | 9.3                                                      | 10.3                                                                     | 11.2                            | 16,000               |
|            | 200 392                    | 8.6                                                      | 9.3                                                                      | 10.9                            | 15,500               |
|            | 250 482                    | 8.1                                                      | 8.7                                                                      | 10.7                            | 15,150               |
|            | 300 572                    | 7.6                                                      | 8.0                                                                      | 10.5                            | 14,950               |
|            | 350 662                    | 7.3                                                      | -----                                                                    | 10.4                            | 14,750               |
|            | 400 752                    | 7.0                                                      | -----                                                                    | 10.3                            | 14,650               |
| 35         | Steel Type                 | Avesta 832 SK,<br>SIS 2343                               |                                                                          | Werkstoff 4436                  |                      |
|            |                            | Swedish Pressure Vessel Code                             | AD-Merkblatt W2 Streckgrenze $\times \frac{2}{3}$ , kg./mm. <sup>2</sup> | ASME Code (Interpolated values) | Kg./mm. <sup>2</sup> |
| 40         | Temperatures               | $\sigma_{ber} \times \frac{2}{3}$ , kg./mm. <sup>2</sup> | $\times \frac{2}{3}$ , kg./mm. <sup>2</sup>                              |                                 |                      |
|            | °C. °F.                    |                                                          |                                                                          |                                 |                      |
|            | 20 68                      | 14.0                                                     | 14.7                                                                     | 13.2                            | 18,750               |
|            | 50 122                     | 12.6                                                     | 13.0                                                                     | 13.2                            | 18,750               |
|            | 100 212                    | 10.8                                                     | 11.3                                                                     | 13.1                            | 18,600               |
|            | 150 302                    | 9.7                                                      | 10.3                                                                     | 12.6                            | 17,900               |
|            | 200 392                    | 9.0                                                      | 9.3                                                                      | 12.3                            | 17,500               |
|            | 250 482                    | 8.5                                                      | 8.7                                                                      | 12.1                            | 17,250               |
|            | 300 572                    | 8.0                                                      | 8.0                                                                      | 12.0                            | 17,100               |
|            | 350 662                    | 7.7                                                      | -----                                                                    | 12.0                            | 17,100               |
|            | 400 752                    | 7.3                                                      | -----                                                                    | 11.9                            | 16,900               |
| 45         | Steel Type                 | Avesta 832 SK,<br>SIS 2343                               |                                                                          | Werkstoff 4436                  |                      |
|            |                            | Swedish Pressure Vessel Code                             | AD-Merkblatt W2 Streckgrenze $\times \frac{2}{3}$ , kg./mm. <sup>2</sup> | ASME Code (Interpolated values) | Kg./mm. <sup>2</sup> |
| 50         | Temperatures               | $\sigma_{ber} \times \frac{2}{3}$ , kg./mm. <sup>2</sup> | $\times \frac{2}{3}$ , kg./mm. <sup>2</sup>                              |                                 |                      |
|            | °C. °F.                    |                                                          |                                                                          |                                 |                      |
|            | 20 68                      | 14.0                                                     | 14.7                                                                     | 13.2                            | 18,750               |
|            | 50 122                     | 12.6                                                     | 13.0                                                                     | 13.2                            | 18,750               |
|            | 100 212                    | 10.8                                                     | 11.3                                                                     | 13.1                            | 18,600               |
|            | 150 302                    | 9.7                                                      | 10.3                                                                     | 12.6                            | 17,900               |
|            | 200 392                    | 9.0                                                      | 9.3                                                                      | 12.3                            | 17,500               |
|            | 250 482                    | 8.5                                                      | 8.7                                                                      | 12.1                            | 17,250               |
|            | 300 572                    | 8.0                                                      | 8.0                                                                      | 12.0                            | 17,100               |
|            | 350 662                    | 7.7                                                      | -----                                                                    | 12.0                            | 17,100               |
|            | 400 752                    | 7.3                                                      | -----                                                                    | 11.9                            | 16,900               |

The following three examples compare resulting wall thicknesses for calculations according to the Swedish, German and United States codes.

### Example III

#### Thin-walled shell:

Design pressure—12 kg./cm.<sup>2</sup> = 171 p.s.i.

Inside diameter—2000 mm. = 78 $\frac{3}{4}$  inches

Working temperature—20° C. = 68° F.

Material—Avesta 832 MV corresponding to SIS 2333, AISI 304, Werkstoff 4301

The required wall thicknesses of the steel according to the different codes in unstretched and cold stretched state will be as follows:

|                                                                   | Sweden                                       | Germany                                      | United States                             |
|-------------------------------------------------------------------|----------------------------------------------|----------------------------------------------|-------------------------------------------|
| Maximum allowable stress according to code                        | $\frac{20}{1.5} = 13.3$ kg./mm. <sup>2</sup> | $\frac{22}{1.5} = 14.7$ kg./mm. <sup>2</sup> | 18,750 p.s.i., 13.2 kg./mm. <sup>2</sup>  |
| Minimum thickness of unstretched shell                            | 0.2 mm.                                      | 8.2 mm.                                      | 0.36 inch, 9.1 mm.                        |
| Yield strength of cold stretched material                         | 35.0 kg./mm. <sup>2</sup>                    | 35.0 kg./mm. <sup>2</sup>                    | 35.0 kg./mm. <sup>2</sup> , 49,780 p.s.i. |
| Minimum thickness of cold stretched shell                         | 5.7 mm.                                      | 5.1 mm.                                      | 0.20 inch, 5.1 mm.                        |
| Reduction in wall thickness when using the cold stretching method | 38%                                          | 38%                                          | 44%                                       |
| Cold stretching pressure                                          | 20.0 kg./cm. <sup>2</sup>                    | 18.6 kg./cm. <sup>2</sup>                    | 18.2 kg./cm. <sup>2</sup> , 280 p.s.i.    |

## 11

## Example IV

## Thin-walled shell:

Design pressure—4 kg./cm.<sup>2</sup>=57 p.s.i.  
 Inside diameter—6000 mm.=236.22 inches  
 Working temperature—100° C.=212° F.  
 Material—Avesta 832 SK corresponding to SIS 2343,  
 AISI 316, Werkstoff 4436.

In this case the working temperature is 100° C.=212° F. However, for practical reasons cold stretching is carried out at room temperature. This means that the material has to be cold stretched to a higher yield strength than the one applicable at the working temperature. As mentioned in connection with Example II, the increase in yield strength obtained at room temperature remains substantially unchanged at higher temperatures. Therefore the required yield strength value at room temperature is calculated by adding the desired increase in yield strength at working temperature to the value applicable at room temperature according to the code.

Based on the values applicable in Sweden the calculation would consequently be as follows:

Yield strength at room temperature:

$$(32.0 - 16.2) + 21.0 = 36.8 \text{ kg./mm.}^2$$

Based on the German code it would be:

Yield strength at room temperature:

$$(32.0 - 17.0) + 22.0 = 37.0 \text{ kg./mm.}^2$$

The ASME code does not state any yield strength values and for this reason we have used the Swedish values in the calculations for the United States. These values also correspond fairly well to the German values.

The required wall thicknesses of the steel according

|                                                                           | Sweden                                      | Germany                                     | United States                            |
|---------------------------------------------------------------------------|---------------------------------------------|---------------------------------------------|------------------------------------------|
| Maximum allowable stress according to code...                             | $\frac{15.6}{1.5} = 10.4 \text{ kg./mm.}^2$ | $\frac{17.5}{1.5} = 11.7 \text{ kg./mm.}^2$ | 17,040 p.s.i., 24.2 kg./mm. <sup>2</sup> |
| Minimum thickness of unstretched shell.....                               | 67.2 mm.                                    | 51.7 mm.                                    | 1.88 inches, 47.7 mm.                    |
| Yield strength of cold stretched material:                                |                                             |                                             |                                          |
| At 350° C., 662° F.....                                                   | 32.0 kg./mm. <sup>2</sup>                   | 32.0 kg./mm. <sup>2</sup>                   | 38,900 p.s.i., 27.3 kg./mm. <sup>2</sup> |
| At 20° C., 68° F.....                                                     | 38.4 kg./mm. <sup>2</sup>                   | 41.5 kg./mm. <sup>2</sup>                   | 54,500 p.s.i., 38.4 kg./mm. <sup>2</sup> |
| Minimum thickness of cold stretched shell.....                            | 27.2 mm.                                    | 24.1 mm.                                    | 1.18 inches, 30.0 mm.                    |
| Reduction in wall thickness when using<br>the cold stretching method..... | 58%                                         | 53%                                         | 37%                                      |
| Cold stretching pressure.....                                             | 500 kg./cm. <sup>2</sup>                    | 485 kg./cm. <sup>2</sup>                    | 7,700 p.s.i., 540 kg./cm. <sup>2</sup>   |

to the different codes in unstretched and in cold stretched state will be as follows:

If it is desirable to produce pressure vessels that will retain their original shape to a greater extent than the

|                                                                           | Sweden                                      | Germany                                     | United States                             |
|---------------------------------------------------------------------------|---------------------------------------------|---------------------------------------------|-------------------------------------------|
| Maximum allowable stress according to code...                             | $\frac{16.2}{1.5} = 10.8 \text{ kg./mm.}^2$ | $\frac{17.0}{1.5} = 11.3 \text{ kg./cm.}^2$ | 18,600 p.s.i., 13.1 kg./mm. <sup>2</sup>  |
| Minimum thickness of unstretched shell.....                               | 12.3 mm.                                    | 10.6 mm.                                    | 0.36 inch, 9.2 mm.                        |
| Yield strength of cold stretched material:                                |                                             |                                             |                                           |
| At 100° C., 212° F.....                                                   | 32.0 kg./mm. <sup>2</sup>                   | 32.0 kg./mm. <sup>2</sup>                   | 32.0 kg./mm. <sup>2</sup> , 45,514 p.s.i. |
| At 20° C., 68° F.....                                                     | 6.8 kg./mm. <sup>2</sup>                    | 37.0 kg./mm. <sup>2</sup>                   | 36.8 kg./mm. <sup>2</sup> , 52,200 p.s.i. |
| Minimum thickness of cold stretched shell.....                            | 36.3 mm.                                    | 5.6 mm.                                     | 0.22 inch, 5.6 mm.                        |
| Reduction in wall thickness when using<br>the cold stretching method..... | 49%                                         | 47%                                         | 39%                                       |
| Cold stretching pressure.....                                             | 7.8 kg./cm. <sup>2</sup>                    | 6.9 kg./cm. <sup>2</sup>                    | 6.9 kg./cm. <sup>2</sup> , 98 p.s.i.      |

## Example V

## Thick-walled shell:

Design pressure—250 kg./cm.<sup>2</sup>=3550 p.s.i.  
 Inside diameter—200 mm.=7.9 inches  
 Working temperature—350° C.=662° F.  
 Material—Avesta 832 SKT corresponding to SIS 2343  
 (stabilized), Werkstoff 4573

In the ASME code there are no figures specified for this grade. Because of its high yield strength it seems correct to use the ASME values for a grade with an allowable stress which is as high as possible. In this case AISI 316

vessel of FIGURES 1 and 2, the austenitic stainless steel plates may be cold stretched, cold rolled or otherwise cold worked prior to being welded together. Referring to FIGURE 3, a pressure vessel includes a cylindrical shell 34 enclosed by domed ends 35 and 36. The shell is formed by a number of arcuately bent austenitic stainless steel plates 37 of Avesta 832 MV steel which have been permanently elongated about 5%. This increases the yield strength  $\sigma_{0.2}$  to about 35 kg./mm.<sup>2</sup>. Since this value can be substituted for 20 kg./mm.<sup>2</sup>, the calculating value  $\sigma_{ber}$  for yield strength given in the Code (see Table 2), the vessel wall can be made substantially thinner with great

savings in stainless steel, as shown by the calculations in Examples I to V.

The plates 37 are then welded together along longitudinal joints 38 and circumferential joints 39 using welding electrodes of the same or similar grade steel as the plates 37. The welding heat causes annealing of the welded joints and narrow zones of the plates adjacent to them which must be assigned, therefore, a calculating value  $\sigma_{ber}$  of yield strength of only 20 kg./mm.<sup>2</sup>, even though they have a statistical yield strength of 24 kg./mm.<sup>2</sup>.

To impart to the circumferential and longitudinal welded joints 38 and 39, and the adjacent annealed zones, the same strength characteristics as those of the cold worked plates 37, the finished vessel is subjected to an internal fluid pressure calculated to raise the yield strength of the weldments and annealed zones to 35 kg./mm.<sup>2</sup>. Since such pressure will cold stretch and elongate permanently only the weld joints and the narrow adjacent annealed zones, the overall circumferential change in the vessel will be extremely small and will have a negligible influence on the shape of the pressure vessel.

The yield strength selected to cold stretch the welded vessel may also be higher than that of the prestretched plates, if desired, to insure a vessel of greater uniformity and still provide a reduction in distortion.

Still a further reduction in distortion of the vessel may be obtained if the joints 38 and 39 are welded with electrodes adapted to impart to the weldments the yield strength of the cold worked plates. If the welded joints are produced in this manner, then only the material in the narrow annealed zones of the plates adjacent to the welded joints will be permanently elongated when the calculated pressure is applied to the completed vessel. Although the width of those zones is small, it may be reduced still further by welding in a cold state; i.e., by cooling the welded joints with a stream of air or the like after each welding run. In this manner only an extremely small change in the shape of the vessel is effected by the cold stretching.

It has been found that the selected yield strength should be sufficiently high after cold stretching to provide a permanent elongation of the austenitic stainless steel in the weakest regions of the pressure vessel essentially in excess of 0.2%. Experiments have shown that which the presently used austenitic stainless steels shown in Tables 1 and 2, the yield strengths selected have most often provided permanent elongations of the weakest regions of the pressure vessels on the order of 1 to 4%. However, higher yield strengths resulting in greater percentages of permanent elongations may also be selected so long as the permanent elongation is at most 10%, for reasons which will be explained in greater detail hereinafter.

With respect to the extent of permanent elongation of the austenitic stainless steel, considering the curves of FIGURES 4A and 4B, note the initial extremely high rate of increase in yield strength of Avesta 832 SK steel up to about 0.365% strain and then the less steep but still high rate of increase. In other words, a permanent elongation of 0.2% requires a strain of about 0.365%, as shown in FIGURE 4B, and encompasses the steepest rise of the curve which must be used to obtain the benefits of the invention. The rate of increase following 0.365% is also high, see FIGURE 4A, and may be used but only up to at most about 10% elongation.

The upper limit of cold stretching austenitic stainless steels is critical because, if exceeded, the ratio of yield strength ( $\sigma_{0.2}$ ) to ultimate tensile strength will increase beyond about 0.8, the upper limit of that ratio required for safety. Referring to the curves shown in FIGURE 6, the ultimate tensile strength and yield strength of grade AISI 316 stainless steel are shown when cold stretched with reference to the cross-section of the original unstretched material. Note that the yield strength ( $\sigma_{0.2}$ ) of the austenitic stainless steel increases at a high rate dur-

ing the first 10% elongation, this also being obvious from the curves of FIGURES 4A and 4B. This high rate of yield strength increase enables the margin between the normal working stress to which the vessel is subjected and the yield strength to remain at a safe level even though the pressure vessels have walls substantially thinner than those previously thought acceptable.

FIGURE 6 also shows that if the austenitic stainless steel is stretched no more than about 10%, the material will still yield sufficiently when subjected to an overload to meet safety standards because the ratio of yield point to ultimate tensile strength will not exceed 0.8 (68,000 p.s.i./85,000 p.s.i.). This is the maximum ratio permitted by safety standards and represents a critical value insofar as consequences are concerned, as does the permanent elongation of about 10% upon which it depends. Of course different melts of AISI 316 steels, and other austenitic stainless steels, have slightly different properties; thus a permanent elongation of 10% might for some provide a ratio of .77, and for others .82, and those differing properties must be considered when selecting the maximum amount of cold stretching to which the vessel will be subjected.

The upper limit of 10% is also important as regards 25 the stress corrosion resistance of austenitic steels. Originally the inventive cold stretched vessels were considered unacceptable by the regulatory authorities due to the deep-rooted conviction that the susceptibility of austenitic stainless steels to stress corrosion increases if 30 such steels are subjected to cold-working. Sections of previous pressure vessel codes, which do not permit testing of stainless steel vessels at pressures 50% greater than their working pressures (ferritic vessels are so tested) to avoid any possibility of cold working the stainless 35 steel, reflect this conviction as well as the prior literature and attitudes in the art of stainless steel. However, extensive tests carried out in connection with the present invention show that cold-working essentially in excess of 0.2% and at most about 10% does not impair significantly the stress corrosion resistance of austenitic stainless steels and, in fact, in certain instances improves their stress corrosion characteristics.

In one test, the results of which are shown in FIGURE 7, from 15 mm. thick plates of Avesta 832 MV and Avesta 832 SK steels that had been cold stretched 0, 2.5, 5 and 10%, specimens were taken partly for corrosion tests and partly for determining the yield strength of the cold stretched steel. Comparative tests were carried out in 40%  $\text{CaCl}_2$ , pH 6 and 100° C. under uniaxial tensile stress. The tensile stress was chosen in relation to the yield strength at 100° C. so that in all cases it amounted to  $\frac{2}{3}$  of the yield stress ( $\sigma_{0.2}$ ). A similar test was carried out with specimens from the same plates that had been welded and then cold stretched and cut so that the central part consisted of weld metal.

One curve in FIGURE 7 shows the characteristics of Avesta 832 SK steel when cold stretched 0, 2.5, 5 and 10%. Also shown is another curve for a welded specimen. The similar results shown are obtained when the weld filler metal is alloyed at least equally or preferably alloyed somewhat higher than the base metal.

It is important to note that the specimens of FIGURE 7, cold stretched to different percentages, should not be tested under the same load but under a load which is 65 proportional to the yield strength at 100° C. An experiment using the same loading stress would not give results as useful as these since the intention is to use the effects of raising the yield strength by cold stretching to decrease the wall thickness of the vessel and increase the stresses in the wall as compared to an unstretched vessel.

FIGURES 8 and 9 show the results of another stress corrosion test series conducted on grade Avesta 832 MV; i.e., non-molybdenum alloyed steel. In this test the corrosion has been accelerated and it can be seen from FIGURE 8 that the time to fracture increases with increasing

degree of cold stretching at identical loads up to about 10%.

The lower curve of FIGURE 9 shows the time to fracture for unstretched specimens while the upper curve shows the time to fracture for stretched specimens. It is apparent that the unstretched steel is inferior to the cold stretched steel with regard to stress corrosion resistance.

In still another stress corrosion test series conducted with welded vessels cold stretched at different internal pressures to different degrees of elongation, the results showed that the unstretched vessels have gone to fracture in considerably shorter time than the cold stretched ones, which is in agreement with the above tests. The failure always occurred near the longitudinal weld of the shell in the unstretched vessels whereas in the cold stretched vessels, the failure always occurred in material that was not influenced by welding. Most probably this can be explained by the fact that the high stresses normally resulting at the weldment have an unfavorable influence on resistance to stress corrosion. These stresses are relieved during the cold stretching; consequently, this is still another advantage derived from the present invention.

The pressure vessels formed pursuant to the present invention have the same resistance to general and intergranular corrosion as do unstretched vessels. Experiments using the Huey test (boiling 65% HNO<sub>3</sub>) have shown that the austenitic stainless steels can be cold stretched 10% without impairing their resistance to such corrosion. In non-oxidizing corrosive solutions (boiling 2% H<sub>2</sub>SO<sub>4</sub>+3% Na<sub>2</sub>SO<sub>4</sub>) cold stretching to 10% does not affect the rate of general and intergranular corrosion.

Moreover, the susceptibility to pitting of the inventive pressure vessels have not been impaired by cold stretching up to 10%; this was proved by tests using acid (10% FeCl<sub>3</sub>, 50° C.) and neutral chloride solutions (4% NaCl+0.2% K<sub>3</sub>Fe(CN)<sub>6</sub>, 25° C.).

Extensive tests have also shown that austenitic stainless steel pressure vessel embodying the principle of the invention have excellent fatigue strength. Six test vessels of Avesta 832 SK stainless steel having a diameter of 400 mm. and a wall thickness of 4 mm. were filled with salt solution and subjected to pulsating inner pressure at a temperature of 150° C. The solution contained 15.5 grams NaCl per liter of distilled water; the solution was aerated prior to testing. Two of the six vessels were constructed of normal stainless steel, two were cold stretched 2% and two were cold stretched 5%. The maximum number of load changes used in this test series was 50,000.

One vessel in each group was subjected to a maximum stress equal to the stress permissible in calculations according to the Swedish Pressure Vessel Code. The other vessels were subjected to higher maximum pressures so chosen that the resulting stress conformed to the calculating value of the Code. In other words, in this case the stress was equal to the value to be used when dimensioning a pressure vessel with a safety factor and a joint efficiency equal to one.

After the above test series were concluded without any material difficulties resulting, the 2% stretched vessel that had been subjected to the highest maximum pressure was then subjected to 55,000 more load changes under the same conditions. Thereafter the pressure was increased so that the maximum stress corresponded approximately to the original yield strength of the material, in this case about 29 kg./mm.<sup>2</sup>; i.e., 85% of the yield strength of the 2% stretched material. Following another 44,000 load changes the test series was interrupted due to failure of the testing equipment.

Thorough laboratory investigations of the vessels thus tested were made and no change could be found. In these investigations special attention was paid to the nozzles and weld points in the vessels.

From the foregoing it is apparent that the invention provides austenitic stainless steel pressure vessels having walls greatly reduced in thickness in comparison to the

wall thickness previously required, thereby affording great savings in the amount of stainless steel used. It will be apparent that the above-described embodiments of the invention are illustrative only and modifications thereof will occur to those skilled in the art.

I claim:

1. In the manufacture of welded pressure vessels from plates of austenitic stainless steel, the method comprising the steps of welding together a plurality of plates of austenitic stainless steel having a normal yield strength with weldments of austenitic stainless steel to form a pressure vessel, selecting a higher than normal value of yield strength within a range of values provided by cold stretching the steel an amount sufficient to elongate it 10 permanently essentially in excess of 0.2% and at most about 10%, and subjecting the vessel internally to a fluid pressure sufficient to stress the weakest portions of the vessel walls to the selected yield strength and thereby increase the yield strength of the said weakest portions to 15 the selected value by permanently elongating the said weakest portions of the walls essentially in excess of 0.2% and at most about 10%, the vessel being subjected to the fluid pressure at a temperature below the recrystallization temperature of the steel and under conditions 20 permitting the vessel walls to expand freely.
2. In the manufacture of welded pressure vessels from plates of austenitic stainless steel, the method comprising the steps of selecting a higher than normal value of yield strength within a range of values provided by cold 30 stretching the steel an amount sufficient to elongate it permanently essentially in excess of 0.2% and at most to a percentage at which its yield strength is increased to a value that provides a ratio of yield strength to ultimate tensile strength of .8, welding together a plurality of 35 plates of austenitic stainless steel with weldments of austenitic stainless steel to form a pressure vessel, and subjecting the vessel internally to a fluid pressure sufficient to stress the weakest portions of the vessel walls to the selected yield strength and thereby increase the yield 40 strength of the said weakest portions to the selected value by permanently elongating the said weakest portions of the vessel walls an amount essentially in excess of 0.2% and at most to a percentage at which the yield strength of the said weakest portions is increased to a value that provides a ratio of yield strength to ultimate tensile 45 strength of .8, the vessel being subjected to the fluid pressure at a temperature below the recrystallization temperature of the steel and under conditions permitting the vessel walls to expand freely.
3. In the manufacture of welded pressure vessels from plates of austenitic stainless steel, the method comprising the steps of selecting a higher than normal value of yield strength within a range of values provided by cold stretching the steel an amount sufficient to elongate it 50 permanently essentially in excess of 0.2% and at most about 10%, welding together a plurality of plates of austenitic stainless steel with weldments of austenitic stainless steel to form a pressure vessel, and subjecting the vessel internally to a fluid pressure sufficient to stress the 55 weakest portions of the vessel wall to the selected yield strength and thereby increase the yield strength of the said weakest portions to the selected value by permanently elongating the said weakest portions of the vessel walls an amount essentially in excess of 0.2% and at most about 10%, the vessel being subjected to the fluid pressure at a temperature below the recrystallization temperature of the steel and under conditions permitting the vessel walls to expand freely.
4. In the manufacture of welded pressure vessels from austenitic stainless steel plates, the method comprising the 60 steps of selecting a higher than normal value of yield strength within a range of values provided by cold stretching the steel an amount sufficient to elongate it permanently essentially in excess of 0.2% and at most about 10%, cold working the steel plates to stress their 65

weakest portions to the selected yield strength and thereby increase the yield strength of the said weakest portions of the plates to the selected value by permanently elongating the said weakest portions of the plates essentially in excess of 0.2% and at most 10%, welding the cold worked-plates together with weldments of austenitic stainless steel to form the pressure vessel, and subjecting the vessel internally to a fluid pressure sufficient to stress the weakest portions of the vessel walls to the selected yield strength and thereby increase the yield strength of said weakest portions to the selected value by permanently elongating the said weakest portions essentially in excess of 0.2% and at most 10%, the vessel being subjected to the fluid pressure at a temperature below the recrystallization temperature of the steel and under conditions permitting the vessel walls to expand freely.

5. In the manufacture of welded pressure vessels from austenitic stainless steel plates, the method comprising the steps of selecting a first higher than normal value of yield strength within a range of values provided by cold stretching the steel an amount sufficient to elongate it permanently essentially in excess of 0.2% and at most about 10%, cold working the plates to stress their weakest portions to the selected first value of yield strength and thereby increase the yield strength of the said weakest portions of the plates to the selected first value by permanently elongating the said weakest portions of the plates essentially in excess of 0.2% and at most 10%, welding the cold-worked plates together with weldments of austenitic stainless steel to form the pressure vessel, selecting a second higher than normal value of yield strength within said range of values, and subjecting the vessel internally to a fluid pressure sufficient to stress the weakest portions of the vessel walls to the selected second value of yield strength and thereby increase the yield strength of said weakest portions of the vessel walls to the selected second value by permanently elongating the said weakest portions essentially in excess of 0.2% and at most 10%, the vessel being subjected to the fluid pressure at a temperature below the recrystallization temperature of the steel and under conditions permitting the vessel walls to expand freely.

6. The method defined in claim 5 wherein the selected

second value of yield strength is higher than the selected first value of yield strength.

7. An austenitic stainless steel pressure vessel comprising a plurality of stainless steel sections, austenitic stainless steel weldments joining the steel sections to form the vessel, the steel sections and the weldments having been stressed to a selected value of yield strength higher than the normal yield strength of the steel by subjecting the vessel internally to fluid pressure sufficient to cause a permanent elongation in the weakest portions of the sections and weldments essentially in excess of 0.2% and at most about 10%, the vessel having been subjected to the fluid pressure at a temperature below the recrystallization temperature of the steel and under conditions permitting the vessel walls to expand freely.

8. An austenitic stainless steel pressure vessel comprising a plurality of stainless steel sections that have been cold worked to elongate them permanent essentially in excess of 0.2% and at most 10%, austenitic steel weldments joining the cold worked steel sections to form the vessel, the steel sections and the weldments having been stressed to a selected value of yield strength higher than the normal yield strength of the steel by subjecting the vessel internally to fluid pressure sufficient to cause a permanent elongation in the weakest portions of the sections and weldments essentially in excess of 0.2% and at most about 10%, the vessel having been subjected to the fluid pressure at a temperature below the recrystallization temperature of the steel and under conditions permitting the vessel walls to expand freely.

#### References Cited

##### UNITED STATES PATENTS

|    |           |         |          |          |
|----|-----------|---------|----------|----------|
| 35 | 2,337,247 | 12/1943 | Kepler.  |          |
|    | 2,579,646 | 12/1951 | Branson  | 29—421   |
|    | 2,652,943 | 9/1953  | Williams | 220—3    |
|    | 2,961,530 | 11/1958 | Macha.   |          |
|    | 2,914,346 | 11/1959 | Ryder    | 29—482 X |

40 RAPHAEL H. SCHWARTZ, Primary Examiner

U.S. Cl. X.R.

29—471.1, 475, 487, 488

UNITED STATES PATENT OFFICE  
CERTIFICATE OF CORRECTION

Patent No. 3,456,831 Dated July 22, 1969

Inventor(s) Johan Ingvar Johansson

It is certified that error appears in the above-identified patent and that said Letters Patent are hereby corrected as shown below:

Column 7, line 1, "According" should read --Accordingly--;

Column 11, fifth line in the last table, "6.8 kg./mm.<sup>2</sup>"

should read --36.8. kg./mm.<sup>2</sup>--;

sixth line in the last table, "36.3 mm." should  
read --6.3 mm.--

Column 15, line 33, "have" should read --has--;

line 39, "trengh" should read --strength--;

line 70, "change" should read --damage--;

Column 18, line 18, "permanent" should read --permanently--.

SIGNED AND  
SEALED  
MAY 5 1970

(SEAL)

Attest:

Edward M. Fletcher, Jr.

Attesting Officer

WILLIAM K. SCHUYLER, JR.  
Commissioner of Patents